

June 18, 1963

R. E. JOHNSON ET AL  
METHOD OF PRODUCING GALLIUM OR ALUMINUM  
ARSENIDES AND PHOSPHIDES  
Filed Dec. 11, 1959

3,094,388

Fig. 1.



Fig. 2.



Fig. 3.



INVENTORS

Rowland E. Johnson &  
Edward W. Mehal

BY *Stevens, Davis, Miller & Wafer*  
ATTORNEYS

**1**

3,094,388

**METHOD OF PRODUCING GALLIUM OR ALUMINUM ARSENIDES AND PHOSPHIDES**  
Rowland E. Johnson and Edward W. Mehal, Dallas, Tex.,  
assignors to Texas Instruments Incorporated, Dallas,  
Tex., a corporation of Delaware  
Filed Dec. 11, 1959, Ser. No. 859,060  
4 Claims. (Cl. 23—204)

This invention relates to a new method of producing compound semiconductors and in particular to the production of gallium arsenide.

Compound semiconductors are customarily produced by a variety of methods. For instance, gallium arsenide is customarily produced by reacting liquid gallium with arsenic in the vapor stage at a temperature at least as high as the melting point of gallium arsenide. However, this method has the disadvantage of requiring a relatively high temperature which increases the susceptibility toward contamination. In addition, this method is not readily adaptable as a continuous production process.

In an effort to overcome the above-mentioned disadvantages, it has been suggested that gallium arsenide be prepared by reducing gallium oxide with a gaseous stream of heated hydrogen and arsenic vapors. Another suggested technique has been to volatilize gallium and arsenic and thereafter codeposit on a relatively cooled surface to form the gallium arsenide.

Each of the above-mentioned techniques, as well as other techniques known to the art, are subject to their own difficulties. The hydrogen reduction of gallium oxide is difficult to complete, and the resulting compound semiconductor is heavily contaminated with oxygen. Similarly codeposition of gallium and arsenic is unusually difficult to control because of the difference in volatility of the two ingredients.

The object of the instant invention is to provide an improved process for production of compound semiconductors and especially gallium arsenide.

Other objects and advantages of the instant invention will be apparent from the description which follows when taken with the drawings in which:

FIGURES 1 to 3 schematically illustrate the best modes for performing the method of the invention.

Briefly stated, the instant invention involves the process of simultaneous reduction of a halide of a group III element and a halide of a group V element. In a preferred embodiment, the invention involves producing the compound semi-conductor by the vapor phase reduction of arsenic halide by hydrogen in the presence of gallium halide or metallic gallium under conditions whereby the gallium arsenide is stoichiometrically produced.

According to one mode of the instant invention, a mixture of arsenic trichloride and gallium trichloride is introduced into a stream of hydrogen in excess of that required for complete reduction of the chlorides. The gaseous mixture is then passed through a hot reaction zone, at for example about 1,000° C. It is theorized that in the hot reaction zone the hydrogen reduces the arsenic trichloride to free arsenic. The combination of high temperatures and low partial pressure keep the arsenic in the vapor phase. It is thought that the gallium trichloride reacts with the hydrogen to form gallium dichloride. An important feature of this invention is that free gallium is not formed in the hot reaction zone. Any free gallium produced immediately reacts with the various chlorides present to form a chloride of gallium which is reduced to the more stable gallium dichloride. There is no gallium arsenide deposited because under

**2**

these conditions, any gallium arsenide produced would be unstable.

Thereafter, the gases are passed into contact with a relatively cool surface maintained at a temperature of from about 200 to 900° C. The gallium dichloride disproportionates and the gallium combines with the free arsenic to form gallium arsenide which deposits in solid form. It is important to note that the deposition temperature is still high enough to maintain the other components of the gas stream in vapor phase, namely, hydrogen and hydrogen chloride which are gaseous even at room temperature, and unreacted gallium and arsenic chlorides as well. Thus, pure gallium arsenide is deposited. Desirably, the temperature of the crystals is maintained high enough to also keep any excess arsenic from depositing on the crystal product.

An extremely close control of product purity is possible when the compound semiconductor is produced in accordance with the process of the present invention. Due allowance for the relative volatility of the gallium and the arsenic in vapor phase at the relatively cool condensation point can be made by employing arsenic in slight excess so that a slight amount of arsenic can remain in the vapors at the condensation temperature and not thereby upset the stoichiometric ratio required for gallium arsenide. Similarly, a measure of control is afforded by variation in the reaction temperature and the condensation temperature or by operating at a higher or lower hydrogen gas pressure and even the ratio of hydrogen to reactants.

Although the above-described process embodies important advantages, it has been found that the utilization of gallium trichloride as an initial constituent presents problems in that gallium trichloride readily hydrolyzes with moisture and is very corrosive. In a second embodiment of the invention, such problems are minimized by forming the gallium trichloride in the reaction chamber. According to this second mode, the gaseous stream which contains only the hydrogen and arsenic trichloride is passed into contact with liquid gallium heated to 900–1100° C. At this reaction temperature, the arsenic trichloride is reduced by the hydrogen to elemental arsenic vapors and HCl. The HCl produced when the  $AsCl_3$  is reduced reacts with the liquid gallium to produce gallium trichloride. This reaction continues until all of the gallium is converted to gallium trichloride. Gallium arsenide is then produced by the same mechanism described in the first embodiment of the invention.

Although the foregoing description has been largely given in terms of the production of gallium arsenide, it should be noted that other compound semiconductors can be similarly produced by employment of other combinations of reactants such as aluminum bromide and phosphorous to produce aluminum phosphide, etc.

For a further understanding of the invention, the following specific examples are presented.

*Example I*

Apparatus as shown in FIGURE 1 is used. The apparatus consists of a quartz tube 10 (25 mm. O.D.; 22 mm. I.D.) having an inlet 11 connected to a suitable hydrogen supply and an exhaust outlet 12. Heaters 14 and 15 are provided to maintain the temperatures noted in the legend. A flask 18 terminating in a dripper 20 is positioned in a branch tube 22 adjacent one end of tube 10. In conducting the process of the invention, hydrogen is admitted through inlet 11 at about 100 cc./min. (0.0045 mole/min.). The flask 18 contains a mixture of  $GaCl_3$  and  $AsCl_3$  in the weight ratio of 37.5 to

50. The dripper 20 is controlled to give a drip rate of about 0.2 cc./min. corresponding to about 0.44 g./min. (average specific gravity 2.2) and about 0.00244 mole/min., assuming an average molecular weight of 180. This gives a mole ratio in the reaction zone of

$$\frac{H_2}{x} = 1.84$$

where  $x$  equals  $GaCl_3$  and  $AsCl_3$ . Gallium arsenide is deposited in the region of tube 10 within heater 15.

*Example II*

Apparatus as shown in FIGURE 2 is used. The tube 30 is the same as tube 10. A flask 32 attached to tube 30 contains  $AsCl_3$  at 100° C. A flask 34 similarly attached contains  $GaCl_3$  at 100° C. Hydrogen is blown through the two flasks at about 400 cc./min. to cause a vapor pressure of 20 mm. for  $GaCl_3$  and 400 mm. for  $AsCl_3$ . The mole ratio of  $AsCl_3$  to  $GaCl_3$  is 20 to 1 and of  $H_2/x$  (where  $x$  is  $AsCl_3$  plus  $GaCl_3$ ) is 2.5. Gallium arsenide is deposited in the rightmost region of tube 30.

*Example III*

Apparatus as shown in FIGURE 3 is used. A tube 40 like tubes 10 and 30 is employed. A flask 42 is attached at one end of tube 40 and contains  $AsCl_3$ . A boat 44 of liquid gallium is located in tube 40. Hydrogen is bubbled through the  $AsCl_3$  and also admitted to the end of tube 40. Hydrogen flow is about 1 liter/min. The mole ratio of  $H_2$  to  $AsCl_3$  is about 76 to 1. Gallium arsenide is deposited at the right end of tube 40.

Although the present invention has been shown and described in terms of the best mode contemplated for carrying out the invention, nevertheless, it will be appreciated that changes and modifications can be made which do not depart from the inventive concepts taught herein. Such changes and modifications are deemed to be within the purview of the invention.

What is claimed is:

1. A method of producing the compound semiconductor gallium arsenide which comprises passing a vapor phase mixture of hydrogen and halides of gallium and arsenic into a high temperature zone maintained at a temperature in the range of from about 900° C. to about 1100° C. to cause the hydrogen to react with the halides producing a reactant stream comprising the halide of gallium as a lower order halide and arsenic in the elemental state, passing the reactant stream produced into contact with a relatively cool surface maintained at a temperature of from about 200° C. to about 900° C. to ensure that the lower order halide of gallium disproportionates releasing part of the gallium in the elemental state and forming the higher order halide of the remaining part of the gallium whereby the elemental gallium combines with the elemental arsenic and condenses on the cool surface as the compound semiconductor gallium arsenide.

2. A method of producing the compound semiconductor aluminum phosphide which comprises passing a vapor

phase mixture of hydrogen, halide of aluminum and phosphorus into a high temperature zone maintained at a temperature in the range of from about 900° C. to about 1100° C. to cause the hydrogen to react with the halide producing a reactant stream comprising the halide of aluminum as a lower order halide and phosphorus in the elemental state, passing the reactant stream produced into contact with a relatively cool surface maintained at a temperature of from about 200° C. to 900° C. to ensure that the lower order halide of aluminum disproportionates releasing part of the aluminum in the elemental state and forming the higher order halide of the remaining part of the aluminum whereby the elemental aluminum combines with the elemental phosphorus and condenses on the cool surface as the compound semiconductor aluminum phosphide.

3. A method of producing the compound semiconductor gallium phosphide which comprises passing a vapor phase mixture of hydrogen, halide of gallium and phosphorus in a high temperature zone maintained at a temperature in the range of from about 900° C. to about 1100° C. to cause the hydrogen to react with the halide producing a reactant stream comprising the halide of gallium as a lower order halide and phosphorus in the elemental state, passing the reactant stream produced into contact with a relatively cool surface maintained at a temperature of from about 200° C. to 900° C. to ensure that the lower order halide of gallium disproportionates releasing part of the gallium in the elemental state and forming the higher order halide of the remaining part of the gallium whereby the elemental gallium combines with the elemental phosphorus and condenses on the cool surface as the compound semiconductor gallium phosphide.

4. A method of producing the compound semiconductor aluminum arsenide which comprises passing a vapor phase mixture of hydrogen and halides of aluminum and arsenic into a high temperature zone maintained at a temperature in the range of from about 900° C. to about 1100° to cause the hydrogen to react with the halide producing a reactant stream comprising the halide of aluminum as a lower order halide and arsenic in the elemental state, passing the reactant stream produced into contact with a relatively cool surface maintained at a temperature of from about 200° C. to 900° C. to ensure that the lower order halide of aluminum disproportionates releasing part of the aluminum in the elemental state and forming the higher order halide of the remaining part of the aluminum whereby the elemental aluminum combines with the elemental arsenic and condenses on the cool surface as the compound semiconductor aluminum arsenide.

References Cited in the file of this patent

UNITED STATES PATENTS

|           |         |              |
|-----------|---------|--------------|
| 2,313,410 | Walther | Mar. 9, 1943 |
| 2,798,989 | Welker  | July 9, 1957 |
| 2,938,816 | Gunther | May 31, 1960 |